

## UNITED STATES PATENT OFFICE

2,008,055

METHOD OF PRODUCING  
FERRO-CHROMIUM

Virgilio Angelini, Milan, Italy

No Drawing. Application April 20, 1932, Serial  
No. 606,530. In Belgium April 28, 1931

## 1 Claim. (Cl. 75—14)

This invention relates to a new and improved method of producing ferro-chromium, which needs no further refining operation, by employing reducing agents such as aluminium, ferro-silicon and calcium-silicide.

It has already been proposed to produce ferro-chromium from chromium ore containing chromium oxide by the employment of exothermic reducing agents such as aluminium, ferro-silicon, and calcium-silicide. It has also been proposed to make use of a mixture of the aforesaid reducing agents for producing the metal alloys in order to obtain special effects in the reduction of metal oxides.

15 I have found that in order to obtain a completely pure product in one operation, thus to be ready for the production of the rustless ferro-chromium it will be necessary to make use of a determined quantitative proportion of the chromium ore and the reducing agents.

According to my invention I employ for the production of ferro-chromium with a high chromium content the following mixture:

65% chromium ore (containing 48% of  $\text{Cr}_2\text{O}_3$ ), 25 23% calcium silicide, 4% aluminium, 4% fluorspar, 2% ferro-silicon and 2% lime.

Making use of the mixture composed as described, I obtain a completely pure product in one operation which needs no further refining operation.

30 If I merely employ a mixture of reducing agents but not in the determined quantitative proportions as indicated above, it is not possible to obtain a product free from all impurities such as excess of the reducing agents.

For carrying out my invention any type of furnace may be used as long as it is capable of keeping in complete fusion the material being used during the whole operation. An electric furnace 40 with electrodes serves the purpose. It is also

possible to use an open furnace; any trough furnace, monophase or three-phase with or without a conducting base similar to that employed in the manufacture of ferro-silicon.

As an example a furnace is fed with a mixture of 1000 kg. composed of: 650 kg. of chromium ore containing 48% of chromic oxide  $\text{Cr}_2\text{O}_3$ , 230 kg. calcium silicide, 40 kg. aluminium, 40 kg. fluorspar, 20 kg. ferro-silicon and 20 kg. lime.

When this mixture has become fluid and reaches the temperature of 1600° C. (operation which requires about one half to two hours) one has already an alloy having a high content of chromium, or to be precise about 60% chromium and about 0.23 carbon, traces of silicon, sulphur and phosphorus, and the rest iron. The quantity of this alloy will be about 240 kg.

If this ferro-chromium is to be used for the production of the rustless chromium iron or rustless chromium steel, it can be introduced into an iron bath, for instance a closed furnace containing 850 kg. fused iron with a carbon content not exceeding 0.1%, the composition of the final product will be of about 0.14-0.16% carbon, 20 12-14% chromium and the rest iron.

In carrying out this second part of the production of rustless chromium iron or steel it is necessary to provide a protective slag, whose composition has for its object the protection of the iron bath from impurities caused by the carbon owing to the contact of the electrodes with the bath.

I claim:

A method of producing ferro-chromium which needs no further refining operation by employing a mixture of exothermic reducing agents characterized by the feature that a mixture is used composed of 65% of chromium ore containing 48% of  $\text{Cr}_2\text{O}_3$ , 23% calcium silicide, 4% aluminium, 4% fluorspar, 2% of ferro-silicon and 2% of lime.

VIRGINIO ANGELINI. 40